

May 10, 1932.

C. G. SHAW

1,858,193

MANUFACTURE OF LEATHER

Filed Feb. 9, 1929

2 Sheets-Sheet 1



INVENTOR  
CHARLES G. SHAW.

BY *Deekastrikingh Co.*  
ATTYS.

May 10, 1932.

C. G. SHAW

1,858,193

MANUFACTURE OF LEATHER

Filed Feb. 9, 1929

2 Sheets-Sheet 2



INVENTOR  
CHARLES G. SHAW.

BY *Deekstra, Haugh & Co.*  
ATTYS.

## UNITED STATES PATENT OFFICE

CHARLES GEORGE SHAW, OF HUNTSVILLE, ONTARIO, CANADA

## MANUFACTURE OF LEATHER

Application filed February 9, 1929. Serial No. 338,876.

This invention relates to improvements in the manufacture of leather with more particular reference to the simultaneous compacting and finishing of pieces of leather, such as vegetable tanned sole leather in pieces such as sides, crops, bends, shoulders and bellies, or any pieces of leather of substantial area as produced at the tannery, and the object of the invention is to devise an improved method 5 or process of simultaneously finishing and compacting such pieces of leather to a desired degree of compactness as may be required for any of the various commercial uses, which improved process results in a 10 finished product of superior quality, finish and value to that produced by methods heretofore used.

In the manufacture of vegetable tanned sole leather there are various classifications, both 20 as to tannage and firmness. Various vegetable extracts as for instance quebracho, chestnut oak, cutch and such like, as well as liquors made from oak, hemlock and wattle bark, and the other vegetable substances, as nuts, shells 25 and such like are used in the tannage of leather and leather tanned outright by the use of these materials is called by various trade names such as vegetable tanned, or oak tanned, or union tanned. Leather of this 30 classification the world over has one quality, which is imparted largely by compacting pressure, that quality is known among the trade on this continent as firmness and is designated throughout British countries usually 35 by the use of such terms as, solid, very solid and firm, or soft as the case may be.

Variations in the actual chemical treatment during the process tend somewhat to 40 modify these qualities in vegetable tanned leather, but the fact remains that rough or unrolled leather, as produced by a single fair average vegetable tannage, that is in such state as exists before it is commonly rolled, may by varying the moisture content and the 45 unit pressures used in the compacting and finishing process, be transformed into any one of the various classifications of firmness as required for sole leather, as for a lady's dancing slipper or a lumberman's caulked sole. It is for the compacting and finishing 50

of vegetable tanned leather in particular that this improved process has been devised although its application in time to come will likely be more varied. This improved process is not intended for use in the manufacture of 55 comparatively uncompacted leather, such as the so called "flexible chrome retanned". Neither will it be of much advantage to use the extremely high unit pressures as in this improved process for the finishing of chrome 60 or mineral sole leather, as the firmness of these tannages is imparted as desired only by changing the nature of the filling material, as by the addition of ceresin wax, resin, or other hard wax to the paraffin base material with 65 which they are usually impregnated. The use of presses in the manufacture of chrome sole leather is for the purpose of obtaining a finished or embossed grain or flesh surface, which may be done at pressures of a few hundred pounds to the square inch of surface, and is not used for the compaction of the leather as is the case in the manufacture of 70 vegetable tanned sole leather by my process.

Furthermore, the faulty finish hitherto so 75 obtained on chrome sole leather could not be tolerated on the vegetable tanned sole leather. Hitherto it has been common practice to finish and compact vegetable sole leather in 80 rolling machines, by means of rolls, usually of the pendulum type or its equivalent, such as flat bed rollers, which rolls are usually, as in America, of comparatively small size although some, as in Great Britain, are of larger size and diameter, but all rolling machines 85 contact at any one time only with a very restricted portion of the surface of the leather and in compacting a piece of leather of substantial area in this way the piece is moved with respect to the roller and its bed so as to 90 eventually cause the roller to work over the entire surface of the piece. When leather is thus compacted by rollers there is a marked tendency to laterally distend the piece and thus unduly thin it. This is not the case in 95 my process, as by exerting a pure squeezing pressure simultaneously over a substantially large area, the surface area is not increased and therefore the sheet is not unduly thinned. Further, when leather is thus 100

rolled due to the lateral distention tendency and the limited area in contact with the roller at any time, the tendency of the fibres to assume the normal (bowed) position in which they grew on the animal, and which is a source of constant trouble and expense to the tanner in the making of a desirably flat piece of leather is aggravated, which is not the case in my process, which produces a desirable sheet-flat piece of leather compacted and finished to any desired degree with the greatest possible ease and in one operation and without the necessity or desirability of rolling.

In France and some other European countries leather has been and is being compacted by hammering which has some advantages, but has not come into use in America and Great Britain due to a great many disadvantages, chief of which are the tediousness and labor cost of the operation and the lack of surface finish produced.

Of the many disadvantages contingent upon rolling the following may be considered among the most important:

25 First. Portions of some hides such as cowhide and Indian buffalo hide hips are badly and unavoidably "bagged", or "cupped". Likewise for instance the rolling of a heavy "finders" bend invariably "dishes" it which is 30 undesirable. These faults as before mentioned, which are aggravated in the rolling process, by my process are corrected and eliminated. In the compacting and finishing by my process of hundreds of thousands of 35 pieces of leather from almost every variety of hide as tanned for sole leather, the percentage which have not been finished with absolute ease to a sheet-like flatness is absolutely negligible.

40 Practically all rolled leather in pieces as bends and crops have a certain amount of dish consequent upon its faulty finishing and compacting. This may be partially removed by prolonged storage in properly 45 built piles, but the fact remains that the majority of leather as shipped from the tannery is "baggy". Chief among many objections to baggy leather are:

A. The difficulty with which it is handled 50 in a dieing out machine while being cut for soles, etc. There have no doubt been hundreds of fingers and thumbs lost by the operators of these machines, which losses might be directly traceable to "baggy" leather. 55 Leather finished by my process lies on the block of a dieing out machine sheet-like in its flatness and allows an operator every possible freedom in the placing of his dies. This one point alone has in at least one cut sole establishment to my knowledge when cutting sheet-flat leather as produced by my process as against a rolled finished leather, increased the efficiency of the dieing out machines and operators by at least twenty-five percent. 60 Further the dies rest normally in a level posi-

tion in cutting sheet-flat leather and do not slide so as to injure the finish or grain when the sole is stamped out and the operator has no reasonable excuse for "dragging his die" or for damaging the grain as is often 70 the case when cutting baggy leather.

B. Baggy rolled finished leather when stripped as for a Knox sole cutting machine causes many of the finest quality strips to be wider across the center than across the ends or "podded". This results in unevenness in the length of soles cut from these strips, or as is usually done prior to cutting the strips into soles, an evening strip is cut from the strip. These trimming strips are called "whip so lashes" in the trade and are wasted. In any case this unevenness in the strips or soles cut from baggy leather is very undesirable and wasteful. Sheet-flat leather as produced by my process is admirably suited for this 75 method of cutting as "podded" strips are eliminated and the soles produced are of even length and the waste of leather for this reason 80 eliminated.

C. Baggy, rolled finished leather does not 85 lend itself to compact parcelling of baling and in storing and particularly ocean shipping this is a decided disadvantage. My process produces leather which stores in less space and bales to the greatest possible compactness and 90 effects valuable saving in the cost of ocean transport.

Second. When branded leather is rolled, the roller in passing over the lump brand, 95 bumps and hammers upon it and makes this part very horny and hard, aggravating the unevenness in texture of these parts. Also rolling does not leave the grain surface of these branded areas level and flat. Further, rolling tends frequently to crinkle the branded area and the lumpy parts are forced in a quite haphazard and uncontrollable manner 100 to appear when finished on either or both the grain or flesh side of the piece; all of which makes the skiving or other subsequent corrective measure very difficult and in many cases impossible to perform. In my process the grain surface is always smooth and flat with the lumps always on the flesh side and all of 105 the disadvantages consequent upon rolling these parts substantially eliminated.

Third. The surface finish as obtained on 110 rolled leather leaves much to be desired as is well known among the trade. By my process a mirror like surface and polish may with 115 the greatest ease be obtained over the whole grain surface of a piece of leather, such as any bend, and the leather may be compacted to any desired degree, all without any rolling, or other finishing process whatever in the 120 space of twenty seconds in one or two strokes of a single machine requiring at this present state of its development only one man to feed the apparatus with leather, and press the button, and another to take it away.

It is, of course, reasonable that the leather should have been previously set out in the normal manner and coarse grained or wrinkled leather should be previously jacked, and this will have a decided tendency to improve the texture and finish of the surface on the completed article, but this preliminary work is not essential to the production, by my process, of a fine and marketable piece of leather. The leather should prior to compacting be properly conditioned as regards moisture content which may be done in any suitable well known way.

Fourth. In all rolling machines there is a decided tendency to exert less pressure on thin portions than on the thicker portions of a piece. For instance, a large proportion of sole leather bends are thinner, over those areas or parts adjacent to the edges where the shoulder and belly have been cut off and these thinner portions are almost invariably of looser fibres than the thicker portions, and require more pressure to suitably compact them. By the use of my process this fault is very easily corrected because they lie at the edges and these thin parts may be given pressures greatly in excess of those applied to other portions, so that a very desirable uniform compactness and feel is given to the whole piece. This is accomplished as herein-after more fully explained:

With the flattening, firming and general improvement in appearance and quality as the object, the pressing of sole leather in pieces such as crops and bends as a supplement to rolling has been tried and has been found of very questionable value due:

Firstly to the variations in thickness in a piece of leather and inequalities such as brands and to the lack of a cushion or other suitable means of properly distributing the pressures over the thicker and thinner portions of the piece in a uniform manner.

Secondly to the great lack of sufficiently high total pressures and to the inadequacy of the apparatus employed to produce them.

Thirdly to the glaring miscalculation or the lack of knowledge and the apparent disregard of the intensity of pressures necessary to accomplish the intended results.

Fourthly to the apparent ignorance of the fact that when leather is once substantially compacted, as in rolling, the fibres become "set" together and a tremendous increase in unit pressure, over the unit pressure used in the rolling is required in a subsequent pressing operation to remove or correct the faults consequent upon or aggravated by the rolling and these extremely high unit pressures were never obtained and properly distributed.

These above mentioned four reasons are illustrative only of many reasons for the practical failure to produce the results claimed of this operation as a supplement to rolling and it must here be stated that any appara-

tus hitherto known in the sole leather industry is so inadequate for the carrying out of my process as to be absurd.

In the above mentioned process of first compacting by rolling and subsequent pressing of sole leather pieces such as are produced at the tannery, no claim such as the one which I now make and claim as my invention had hitherto to my knowledge been made, that leather of suitable tannage for the use it is intended, such as vegetable tanned sole leather in pieces such as bends or crops, may simultaneously be compacted and finished by a pure pressing process in a single machine to any compactness or firmness as required by the sole leather trade and this without the necessity or desirability or use of rolling, which is entirely eliminated, or any other compacting or finishing operation. Furthermore, the leather as produced by my improved process is superior in substantially every respect to like leather finished by any other process hitherto devised. Furthermore, the increased cutting value and superior finish of leather produced by my process is at once apparent and may readily be appraised, and my claim as to the increased value of the product readily substantiated and secondary only to this superior value of the product are the advantages of increased efficiency of the apparatus resulting in the use of fewer machines for compacting purposes, as the rollers may be entirely eliminated, and each machine is of much greater output capacity which results in a saving in valuable factory floor space and makes possible a much more efficient system of routing and handling the material to and from the machines.

Furthermore, the operators for my process need not be highly skilled as is the case in rolling and any intelligent laborer can be taught to operate the apparatus to capacity production in a very short time.

There is also by the use of this process a very substantial reduction in labor costs effected. This in the majority of tanneries may reasonably be expected to amount to fifty percent of the labor costs involved by their present method of compacting. In some tanneries where great care is taken in finishing and the sole leather is rolled two or three times this saving might be much greater. It is of course impossible to make a positive statement in this respect.

Furthermore pigmented films or dressing of such a nature as to not successfully withstand the action of a rolling machine may to great advantage be applied to the leather while the grain is open fibred and absorbent and in such a state as is commonly found in sole leather tanneries, at that stage of the process where it is dry after having been oiled the second time and set out and preferably jacked. These films may be of a waterproof

nature in which case subsequent to pressing, tempering of the leather is effected by putting water, or suitable emulsion on the flesh side and allowing it to "samme" through to the grain side before pressing and this leather is beautifully compacted and finished by this purely pressing process without the necessity or desirability of rolling or any other process whatever, and any degree of compactness desired may be obtained in such leather by the use of my process.

The invention consists in the improved process, all as hereinafter more particularly described. The fundamental intrinsic principle involved is the application of sufficiently high intensities of pressure applied simultaneously over the whole or at least a substantial area of a piece of leather in a purely squeezing and compacting manner, to force the whole or at least a substantial portion of the piece of leather of such dimensions and nature as previously explained, to assume a sheet-like flatness as desired and to exert these sufficiently intense pressures properly distributed, by any suitable apparatus, over the whole of the piece or that substantial part thereof which lies within the apparatus, and a sufficiently high total pressure applied, simultaneously to meet the requirements of the high unit pressures which are necessary to force the previously substantially uncompacted leather fibres to become compacted by this squeezing force to any desired degree as required for marketable sole leather, of any firmness desired; and that during this operation the fibres are so moulded and set by these sufficiently high unit pressures that the piece of leather remains sheet-flat upon its removal from the apparatus. Furthermore by use of an improved apparatus in the nature of a pad or cushion as described hereinafter and in my co-pending application, all irregularities in thickness, and humps, as brands and as found in ordinary marketable sole leather are successfully coped with, and do not cause serious concentrations of pressure on these thicker portions of a piece. As a result of the successful distribution of pressure over the whole surface of the piece, the grain surface of the leather which when quite plastic and which when pressed against the flat mirror-like surface, preferably chromium plated, of the wearing plate acquires during the compacting process the facsimile of the polished surface against which it is pressed. This finish is more easily obtained by properly conditioning the grain as with water or any other suitable wash or dressing prior to pressing.

Likewise the flesh side acquires a very pleasing and marketable appearance from its contact with the smooth spring steel or other top sheet of the pad. Mention has been herein made of the desirability of applying higher unit pressures on thin, loose fibred por-

tions of the leather than on thicker, firmer fibred portions adjacent to them. This may be accomplished most readily by the use of what I have termed a balanced anvil block as illustrated in Fig. 3 in conjunction with the improved pad, which are more fully described in my co-pending application.

This improved process may be successfully carried out in any press of sufficient capacity, platen size, and strength by a proper adjustment of the pad for the control of edge pressures, as by perforating some of the rubber sheets in a suitable manner and adjusting the thickness of the pad by adding a sufficient number of layers of rubber and steel to give ample cushioning action; but the balanced anvil block is of great assistance in relieving the pad of unnecessary work and the press of unnecessary side strains and it should be used. By the use of such an anvil block with a suitable pad upon its surface as in my co-pending application, suitably graded intensities of pressure may be exerted over the whole surface of the piece of leather such as an ordinary bend as follows.

Assume that the dimension of the top surface of the pad and anvil block are 42 inches wide and 72 inches long, and the bend to be pressed is 24 inches wide and 50 inches long and thinner along the belly edge than the back edge and likewise thinner at the shoulder than at the butt end; due to the balancing action of the anvil block any straight line drawn across the top surface of the pad and through the center point, such as center or diagonal lines, will divide the total imposed load according to the laws of leverage such lines acting as fulcra.

Assume that such a bend is placed lengthwise on the surface of the pad so that its center rests upon the center of the pad, then as the press closes the anvil block which is free to align itself, tilts slightly upward on that side upon which the belly side of the bend rests and likewise at that end upon which the shoulder end of the bend rests, really a sort of diagonal tilt. In this manner any tendency of a piece of leather to be thicker at one edge than the opposite edge is in a general way compensated for and during the first stages of the squeeze. All other irregularities in the thickness of the piece are compensated for by the action of the pad, and the bend is thus uniformly pressed with uniformity of intensity of pressure all over its whole surface area.

If, however, the bend is placed lengthwise on the platen as before and moved endwise so that the shoulder edge of the bend is closer to the crosswise center line of the pad than the butt edge then the crosswise center line of the pad does not equally divide either the area or the length of the bend which lies on either side of it, and with the crosswise center line of the pad acting as fulcrum, the butt

part has the advantage of both greater length and area than the shoulder part, and by closing the press and exerting the desired total squeezing pressure on the bend as so placed, 5 that part of the total load which is imposed on the butt part will be less than that part of the total load which is imposed on the shoulder part.

Furthermore, the shoulder part being both 10 of lesser length and area and having imposed upon it a greater portion of the total load than the butt portion will consequently receive much higher intensities of pressures distributed over its smaller area than are distributed 15 over the larger butt area by the lesser portion of the total load and the desired degree of compactness both in the shoulder and the butt parts attained.

Thus by the use of my process in a manner 20 similar to that just described and as in a press capable of exerting from six to ten squeezes per minute, each of five thousand tons or as desired, which speeds and tonnages are readily obtainable, by placing a crop in two or 25 three differing positions on the surface of the pad and by the use of two or three strokes of the press, which strokes may be of varying tonnage as desired, the simultaneous finishing and compacting of a sheet-flat sole or other 30 leather crop may be accomplished with great finesse and dispatch, and without the necessity or the desirability of rolling.

As before mentioned the desirability of 35 having the leather reasonably smooth and free from folds before pressing may be readily understood.

The general appearance, feel and finish of 40 sheet-flat sole leather as finished by my process is very superior and may easily be obtained throughout the whole range of varieties as on the market, turn-sole leather requiring pressures from about two thousand pounds to about thirty-five hundred pounds to the 45 square inch of grain surface area under pressure. Ordinary manufacturer's leather or leather generally suitable for Goodyear sewing requiring from about five thousand to perhaps seven thousand pounds. Firm finishes as for finders' bends requiring from 50 about six thousand pounds to perhaps ten thousand pounds per square inch, although this last figure may be a somewhat low limit and for finishing the extremely hard and firm 55 tannages, such as are admirably suited for caulked soles for river driver's use in the lumber industry, pressures of from fifteen thousand to about twenty-five thousand pounds per square inch may be advantageously employed. The pressure employed for the 60 respective varieties may vary considerably from those noted above, due to variations in the type of hide, and the tannage, but these pressures are substantially accurate. If desired, suitable mechanism may be provided 65 whereby this whole range of pressure is con-

veniently and instantly under the control of the operator. For instance, in the apparatus now in use for carrying out my process this is accomplished by the pressing of an electric control button which shuts the valve supplying the hydraulic press with water and allows the press to open and the total pressure attained at any stage of a stroke is shown on the dial of an ordinary hydraulic gauge. 70

Further, no adjustments whatever are required of any part of the apparatus for the use of any intensity of pressure desired, the pressure is simply switched off when the proper intensity as desired by the operator is attained. 75

Another very important feature of this process is the ease with which the finishes or degrees of compactness are duplicated and standardized, and by varying the conditioning of the leather, and the dressing which may be used and the unit pressures employed during its pressing an astonishing variety of finishes may be produced from the same tannage of leather. 85

As before mentioned these results are not possible of attainment by any apparatus hitherto known or used in the leather industry. The apparatus at present used in my process is capable of exerting in one squeeze a total squeezing pressure of over six thousand nine hundred tons, six times per minute and of properly distributing this high total pressure as may be desirable, and any intensity of pressure up to and even in excess of twenty thousand pounds per square inch may be successfully applied as may be desirable to obtain any degree of compactness required in the product and thus eliminating entirely the process of rolling. 90

In accompanying drawings is shown an apparatus suitable for carrying out the improved process, which apparatus is similar to that described in my co-pending application. 105

In the drawings, 110  
Figure 1 is a diagrammatic sectional elevation of a press suitable for carrying out the improved process.

Figure 2 is a diagrammatic sectional elevation showing a step in the process, the apparatus illustrated in this figure being slightly modified from that illustrated in Figure 1. 115

Figure 3 is a diagrammatic sectional elevation of a modified form of apparatus in which the pad A is supported upon what may be termed a balanced anvil block and in this view is shown a central lengthwise section of an ordinary steer hide bend. 120

Figure 4 is a detached view of the bend shown in Fig. 3. 125

In the drawings like characters of reference indicate corresponding parts in the various figures.

In the apparatus as illustrated, the station- 130

ary head platen of an hydraulic press of suitable strength and capacity is indicated by the numeral 10 and the anvil block or moving platen of the press by the numeral 11 which 5 should preferably, but not necessarily be constructed so as to readily align itself while pressing a piece of leather of wedge shaped cross section such as a stag bend or shoulder and which feature I have called the balanced 10 anvil block as in my co-pending application. A indicates a special form of laminated pad suitable for carrying out my process which pad is composed of layers 12 of spring steel or rawhide alternating with layers 13 of rubber or rubber composition and the layers 13 may, if desired, be provided with perforations 14 or other irregularities of section and the thickness of the layers 12 and 13 of the 15 pad would preferably be of progressively decreasing thickness from the bottom to the 20 top of the pad.

A wearing plate 15 having a suitable surface finish is carried by the head platen 10 and may, if desired, be formed with means 25 for heating the plate such as the steam passages 16.

A piece of leather being operated upon is shown in position within the press by the 30 numeral 17, the piece being so placed that the flesh side thereof contacts with the pad A while the grain side is uppermost so as to come in contact with the wearing plate 15.

In Figure 2, the leather piece 17 which is 35 in position and being pressed is shown as having a blemish or brand mark 18 which causes a hump on the flesh side and this will be later referred to. Also in Figure 2 the perforations have been omitted from the pad A.

In finishing leather according to the 40 improved process the leather piece 17, after it has been so treated that it contains the proper humidity content, which may be done in any suitable well known way, is placed upon the pad A with the grain side uppermost and the 45 piece is then subjected to pressure within the press and in this pressing operation the piece is subjected to a pure pressing action without the desirability or necessity of previous or subsequent rolling and pressures of from 2000 50 pounds per square inch of leather surface upwardly to practically any desired pressure 55 may be successfully employed, which pressures may be very greatly in excess of pressure which could be used when compacting by 60 rolling.

The most important feature of the process 65 is that all or at least a substantial area of the leather piece is subjected simultaneously to a pure pressing operation wherein unit pressures of sufficient intensity are properly distributed over the area under pressure and thus not only is a desirably uniform compactness obtained throughout the area of the piece but the piece is forced to assume a sheet-like flatness and as the fibres are compacted

and set in this position by the high pressures employed the sheet remains flat on its removal from the press.

A further very important feature of the improved process is that blemishes such as 70 brand marks, indicated at 18 in Figure 2, may be successfully coped with and when a piece containing a hump 18 caused by a brand mark is being pressed this hump will cause a depression in the upper layers of the 75 cushion pad A so that the compacting of the piece at the hump will be comparatively uniform with that throughout the remainder of the piece and when the piece is removed from the press this hump may be 80 conveniently skived off from the flesh side so that the blemish so far as is humanly possible may be removed, which makes this blemished portion much less undesirable.

If desired, the wearing plate 15 may be 85 heated, as illustrated in Figure 1, and by this means a more perfect finish may be obtained on the grain side as there is a tendency when the grain side of the leather is warmed while under pressure to soften the 90 leather on this surface so that it tends to flow and the result is a more perfect finish.

Referring to Fig. 3 of the drawings, this shows the provision of a balanced anvil block 19 which is provided with a spherical bearing 20 seating in a spherical set 21 in the platen 11. The pad A is supported upon the anvil block 19 and is positioned thereon so that the center of curvature of the spherical seat is at or near the center of the top 95 surface of the pad and therefore the anvil block and with it the pad is capable of a tilting movement upon the platen 11 in which movement the center point of the top 100 surface of the pad does not move.

In Fig. 3 a steer hide bend 22 is shown in lengthwise section being pressed within the press. This bend is of varying thickness, the shoulder portion B being thinner and of looser fibre structure than the kidney portion C. Also the butt tip D may be either thicker or thinner than the portion C.

If a uniform compactness and firmness is to be produced in the finished bend it is necessary that the unit pressures over the area of the bend be so distributed that the loose fibred portions be subjected to a greater intensity of unit pressure than the closer fibred portions and this distribution of unit pressure must be accomplished regardless of the thickness of the respective portions of the bend.

This desirable distribution of unit pressures is facilitated by the use of the balanced 110 anvil block 19.

In placing a bend 22 in the apparatus shown in Fig. 3, the operator predetermines those portions of the bend which are to be subjected to greatest and least unit pressures 115

and by properly positioning the bend on the surface of the pad A with respect to the centre point thereof when the squeeze is exerted, the anvil block and with it the pad will tilt 5 and due to the principle of levers functioning with the centre point of the top surface of the pad as fulcrum the distribution of unit pressures over the surface of the bend will vary, depending upon the disposition and 10 characteristics of the various local curves of the bend with respect to the centre point of the top surface of the pad.

In this way, by suitably placing the bend as above described, the total load imposed 15 upon the bend may be divided with respect to any straight line passing through the centre point of the top surface of the pad so that by the use of the balanced anvil block described and the resilient pad A the total 20 load is distributed as desired.

From the above it will be apparent that by suitably positioning a bend in the apparatus an infinite variety of loading conditions may be obtained whereby practically 25 any desirable distribution of the total load may be effected to produce the results desired in the finished article.

As previously stated, in carrying out the improved process, unit pressures greatly in 30 excess of those possible in rolling may be readily employed so that greater compactness in the finished product may be obtained, and due to absence of spreading, the thickness of the finished piece is not merely as seriously af- 35 fected, the unit pressure used depending upon the degree of compactness, firmness or hardness of the leather desired in the finished product.

It will be understood that by compacting 40 or compactness is meant the stiffening effect called in the trade "firmness" which firmness has reference to the resilience or resistance to bending, like a sheet of thin spring metal, and also to the ease with which it may be cut, 45 sewn or otherwise worked in a shoe factory. Also, substantially uncompacted leather, means leather not sufficiently compacted or firmly or properly finished to be termed "fin- ished sole leather".

50 In the foregoing specification and appended claims, the term "vegetable tanned sole leather" means sole leather in the tannage of which the chief tanning agent is an extract or liquor of vegetable origin containing tan- 55 nin, or any blend of tanning materials as are commonly known to the trade, and which leather when analyzed in accordance with the official method of the American Leather Chemists Association is shown to contain 60 tannin.

As the sheet-like flatness of the leather as produced by this process is one of its great advantages, in the carrying out of this process, in order to facilitate the attainment of this 65 sheet-like flatness, such machines as may be

used in preliminary operations on the leather should be such as will have a smoothening effect on the leather, such as a jack or setting out machine, without firming the leather, as opposed to machines which have a decided firming effect, such as rolling machines. In other words, it is intended and desired in my process to effect the entire firming of the leather in the pressing operation as described, as this facilitates the production of leather having firmness in any desired degree combined with sheet like flatness. 70

From the foregoing it will be apparent that the invention provides an improved process for the manufacture of sheet-flat leather which will have wide application and by which the objects of the invention have been attained. 75

I believe myself to be the first to recognize not only that leather of the character indicated may be compacted in flat condition by high pressures exerted simultaneously over a substantial area but that tilting of the adjoining faces of a press may be taken advantage of to vary the pressure upon different parts of the leather so that a heavier pressure can be exerted upon a relatively small area, the moment of pressure upon any unit area of the leather with reference to the tilting axis of the face of the anvil being made equal to the moment of the pressure upon any other unit area. 90

I believe myself also to be the first to provide any effective interaction between the press and the leather to assist in making this 100 selective variation in pressure most useful by tiltably mounting (here spherically mounting) one of the platens of my press.

It will be evident that the spherical mounting, as distinguished from mere pivotal mounting, makes the platen adjust automatically about any line through the face of the platen or its adjoining pad and not merely through a single basis line. 105

It will be further evident that the placing 110 of the tilting axis or center close to the surface of the leather being compacted, substantially eliminates lateral movement of the leather during its compaction notwithstanding that the movable platen may re-adjust its position after compacting has begun.

It will further be evident that the selective variance in the pressure above does not in the least interfere with but cooperates with the pressure upon the edges of the leather 120 due to the tension of the margin of the pad caused by sinking of the leather into the pad, and that neither of these benefits interferes with the distribution of pressures in the pad by lumps or extra thicknesses of the leather 125 which may be varied by change in the thickness and other characteristics of the tension plates and elastic filling members used and the extent of progressive variation in their thickness and character. 130

It will be further evident that because the thicker portions of the leather are driven into the pad to a greater extent than the adjoining portions of the leather there will be an action by the marginal portions of the pad about them similar, even if of less degree, to the action about the margin of the leather pressed.

As many changes could be made in the above process and many apparently widely different embodiments of my invention, within the scope of the claims, constructed without departing from the spirit or scope thereof, it is intended that all matter contained in the accompanying specification and drawings shall be interpreted as illustrative and not in a limiting sense.

What I claim as my invention is:—

1. In the manufacture of vegetable tanned sole leather, the steps in the compaction between a die of a press and a cushioning pad in the press of pieces of uneven thickness to substantial uniform firmness, which consists in applying pressure greater than one thousand pounds per square inch, simultaneously to a substantial area of the piece, cushioning the pressure on the flesh side of the leather flexibly in all vertical planes and using cushioning tension at the edge to harden the edges of the leather.

2. The method of simultaneously compacting and finishing substantial areas of vegetable tanned sole leather of unequal thickness, which consists in simultaneously applying compacting pressure of the order of one thousand pounds per square inch or greater to one side of substantially the entire area of a piece of leather while supporting it resiliently and flexibly in all planes perpendicular to the leather to a depth of flexible and resilient support much greater than the difference in thicknesses of leather in the area compressed, whereby abruptness of variation is avoided.

3. The method of simultaneously compacting and finishing substantial areas of vegetable tanned sole leather or the like of unequal thicknesses, which consists in applying compacting pressure of the order of one thousand pounds per square inch or greater to one side of the leather, concurrently pressing it resiliently to different extents, varying directly with the thicknesses, on the other side and distributing the difference in pressure for different thicknesses of leather compressed, progressively by reason of the resilience of the pressure, whereby the area of resilient compression is increased and the extent of compression is reduced as the distance from the thicker parts of the leather increases.

4. The method of simultaneously compacting and finishing substantial areas of vegetable tanned sole leather or the like of unequal thicknesses, which consists in applying compacting pressure of the order of one thousand pounds per square inch and upward, si-

multaneously over a substantial area of the leather between a firm surface and a resilient surface locally yielding in all vertical planes and thus embedding the leather beneath the resilient surface and hence setting up tension in the margin of the resilient surface and tightening the margin against the leather to intensify the pressure at the edge of the leather as compared with the pressure otherwise available there, the pressure conforming to the surface at all points.

5. The method of adjusting the pressure upon a piece of leather being compressed at compacting pressures which consists in shifting the plane of one of the compacting surfaces of the press to partly equalize pressure across the surface while maintaining the lateral position of the compacting surface practically unchanged and in concurrently exerting locally yielding resilient pressure in all planes perpendicular to the leather over a substantial area of the surface of the leather.

6. In the pressing art using a resilient pad made up of highly compressible resilient material between substantially non-compressible flexible sheets, the method which consists in causing a relatively quick initial sagging of the leather into the pad with a rapid stop to the sag by means of perforations in the compressible resilient material at intervals, to provide for local flow of the material initially into the openings provided.

7. The process of transmitting pressure for the purpose of hardening leather which consists in maintaining one side of the leather in a plane, in applying to the other side compacting pressure resiliently and flexibly in all planes vertical to the leather concurrently over a substantial surface of the leather and in distributing the differences in pressure for different leather thicknesses progressively in the backing by which the pressure is applied so that the area of deformation increases and the lateral extent of deformation decreases within the packing as the distance beneath the surface of the packing increases.

8. The method of compacting and finishing substantial areas of vegetable tanned sole leather of unequal thicknesses which consists in maintaining one side of the leather plane, in heating that side of the leather and in concurrently pressing the opposite side of the leather resiliently and flexibly within all planes perpendicular to the surface of the leather throughout a substantial area of said surface.

9. The method of compacting vegetable tanned sole leather or the like which consists in maintaining the grain side of the leather rigidly in a plane and in resiliently applying pressure conforming to the surface at all points upon the flesh side of the leather concurrently throughout the entire surface of the leather.

10. The method of compacting vegetable

tanned sole leather or the like which consists in maintaining the grain side of the leather rigidly in a plane and in resiliently applying pressure of the order of one thousand pounds per square inch or greater concurrently, conforming to the surface at all points throughout the flesh side thereof and varying locally in pressure with the resistance of the leather to compression, progressively greater pressure being applied to thick and firmer parts of the leather than to thin and softer parts of the leather.

11. The method of compacting vegetable tanned sole leather or the like which consists in maintaining the grain side of the leather rigidly in a plane and in resiliently applying pressure conforming to the surface at all points, of the order of one thousand pounds per square inch or greater, concurrently upon every point of the flesh side thereof, which pressure is increased at the edges.

12. The method of compacting vegetable tanned sole leather or the like which consists in maintaining the grain side of the leather rigidly in a plane and in resiliently applying pressure conforming to the surface at all points and of the order of one thousand pounds per square inch or greater to the flesh side of the leather, the moment of pressure upon any unit area of the leather on one side of the press being made equal to the moment of the pressure upon any other unit area and the plane of one of the compacting surfaces being adapted to shift to equalize these pressures.

13. The method of compacting vegetable tanned sole leather or the like which consists in maintaining the grain side of the leather rigidly in a plane and in applying pressure resiliently and of the order of one thousand pounds per square inch or over, concurrently to a considerable area of the flesh side of the leather and of increasingly greater pressures locally to thicker portions of the leather, the pressure conforming to the surface at all points.

14. The method of compacting vegetable tanned sole leather or the like which consists in maintaining the grain side of the leather rigidly in a plane and in applying pressure resiliently of the order of one thousand pounds or greater per square inch, concurrently over a large area on the flesh side while allowing the grain side of the leather to creep in its rigid plane, the pressure conforming to the surface at all points.

In witness whereof I have hereunto set my hand.

CHARLES GEORGE SHAW.